

1,026,733.

F. DE BUIGNÉ.  
PROCESS FOR CASTING METALS.  
APPLICATION FILED OCT. 14, 1911.

Patented May 21, 1912.



Witnesses:

Thomas M. Smith  
Helen J. Miller

Inventor.  
Franz de Buigne,  
By  
J. Walter Douglas  
attorney.

# UNITED STATES PATENT OFFICE.

FRANZ DE BUIGNÉ, OF MAGDEBURG, GERMANY.

## PROCESS FOR CASTING METALS.

1,026,733.

Specification of Letters Patent.

Patented May 21, 1912.

Application filed October 14, 1911. Serial No. 654,781.

*To all whom it may concern:*

Be it known that I, FRANZ DE BUIGNÉ, a subject of the Austro-Hungarian Emperor, and resident of Magdeburg, in the Kingdom 5 of Prussia, German Empire, have invented a new and useful Improved Process for Casting Metals, of which the following is a full, clear, and exact specification.

This invention relates to a process for casting metals under pressure, that is, particularly difficult fusible metals such as iron, 10 bronze, aluminum or the like.

The invention consists in melting the metal by internal heating in a container, or maintaining the metal molten by internal heating in the container, during the casting operation.

Hitherto the casting metals under pressure has generally been effected through external heating. In the event of metals to 20 be cast being of high melting point and when high pressures are used external heating has its disadvantage, is difficult or impossible to keep the walls of the furnace or 25 crucible sufficiently resistant at these high temperatures. According to this invention the heating is from within and in consequence it is possible to keep the outside of the crucible or furnace by choice of suitable 30 constructional material and suitable thickness of wall and if necessary by cooling devices, sufficiently cool to insure the desired degree of resistance to mechanical pressure or gas pressure, such as is unavoidable in the 35 process of casting under pressure, without disturbing the melting operation.

The contents of the crucible may be heated in various ways; for example by introducing a flame of gas under pressure. In many 40 cases it is advantageous to use electrical heating.

In the accompanying drawing the invention is illustrated diagrammatically, a vertical section through an electric furnace being 45 shown by way of example.

*a* is the hearth of the melting and heating chamber, *a'* is the cover, *b* the external casting, *c* the molten bath, *d* and *d'* the electrodes, *e* the delivery pipe for the molten metal, *f* the part of this pipe which is external to the furnace chamber.

*g* is the pipe for the supply of the gaseous pressure medium, *h* is a branch of this pipe and communicates with the atmosphere; *i* is 55 a spring pressed admission valve in the pipe *g*, *k* is a spring pressed exhaust valve in the

branch *h*. Both these valves can be operated in suitable manner, such as by a lever *m*.

With the apparatus shown in the drawing 60 casting is performed as follows:—The solid or molten metal is charged into the melting chamber through an opening not shown in the drawing, and is melted or kept molten with aid of the electrodes *d* and *d'*, which 65 may operate on the arc or resistance principle. The hearth *a*, so far as it comes in contact with the molten metal, consists of material as resistant as possible. In many cases carbon, which may be mixed with refractory clay or the like, is used. The cover 70 *a'* is of any suitable material. The electrodes *d* and *d'* are preferably movable, being made tight by means of stuffing boxes or the like. It is also possible to use the hearth 75 in known manner as one pole, in which case a suitable device for supplying current is provided.

For starting the casting operation, the spring pressed admission valve *i* is opened. 80 The gaseous pressure medium enters the furnace through pipe *g* and forces a certain quantity of the molten metal through the pipe *e*. Against the upper end *f* of the delivery pipe *e*, a suitable mold is pressed. 85 When the spring pressed valve *i* has been closed, the spring pressed valve *k* is opened, whereby pressure is relieved and the casting operation interrupted. The pipe *e* is preferably contracted as shown in the drawing 90 for a length about equal to the height of the furnace and is then expanded up to the delivery end, as shown at *f*. The object is thus achieved that when toward the end of the casting operation a part of the metal in the 95 pipe solidifies, this part can be withdrawn as a lug attached to the object cast. The non-solidified portion of the metal in the delivery pipe returns to the metal bath as soon as the pressure has been relieved. This construction of the delivery pipe does not form a part of this invention.

By opening the spring controlled exhaust valve *k* the compressed gaseous medium is 100 allowed to escape very rapidly from the melting chamber, so that a diminished pressure is produced which exerts a suction on the delivery pipe and draws back the excess of metal into the bath. This action is of 105 particular importance when the delivery pipe is more horizontally placed than as shown in the drawing. Moreover, the sud-

den release of the gas pressure by opening the spring controlled valve *k* may be useful in casting hollow bodies; for if the said valve *k* be opened after the walls of the casting have solidified but before the interior is solid, the liquid metal may be sucked back from the interior of the casting by the aforesaid suction, into the melting chamber. This suction can be aided, if desired, by connecting pipe *h* with a vacuum pipe at the same time that valve *k* is opened.

In many cases it is advantageous that a gas which is indifferent to the molten metal should be used as pressure medium. For instance, nitrogen, carbon dioxide or another gas suitable for the individual case, may be used. This presents the advantage that the electrodes and furnace lining, so far as the latter consists for instance of carbon, are much economized, and the metal bath remains very pure, because oxidation of the bath by the gaseous pressure medium is avoided and the introduction of considerable quantities of electrode ashes are avoided, both of which sources of impurity were hitherto inevitable.

The delivery pipe is shown in the drawing in one position, but according to the kind of object to be cast and the mold to be used, it may have any other upwardly, laterally or downwardly directed position.

By the present process and apparatus large or small objects which may be solid or hollow, may be cast; the whole contents of the metal bath may be used at once for making a correspondingly large article, or only a comparatively small quantity of metal may be used for each casting operation, so that the contents of the furnace suffices for a large number of separate castings; the metal consumed can be made good either continuously or periodically.

What I claim is:

1. In a process of casting molten metals under pressure, which consists in heating a metal bath internally, suddenly releasing the pressure established by an indifferent gas so as to produce by the rapid escape of the gases a partial vacuum in the melting chamber, substantially as and for the purposes described.

2. In a process of casting molten metals under pressure, which consists in heating a metal bath internally by means of electricity, suddenly releasing the pressure established by an indifferent gas so as to produce by the rapid escape of the gases a partial vacuum in the melting chamber, substantially as and for the purposes described.

3. In a process of casting molten metals under pressure, which consists in heating a metal bath internally, suddenly releasing

the pressure established by an indifferent gas so as to produce by the rapid escape of the gases a partial vacuum in the melting chamber and then increasing the vacuum thus created, substantially as and for the purposes described.

4. In a process of casting molten metals under pressure, which consists in heating a metal bath internally by means of electricity, suddenly releasing the pressure established by an indifferent gas so as to produce by the rapid escape of the gases a partial vacuum in the melting chamber and then increasing the vacuum thus created, substantially as and for the purposes described.

5. In a process of casting molten metals under pressure, which consists in heating a metal bath internally by means of electricity, maintaining an atmosphere of an indifferent gas above the molten metal, releasing the pressure to establish a partial vacuum and then increasing the said vacuum, substantially as and for the purpose described.

6. In a process of casting molten metals under pressure, which consists in heating a metal bath internally by means of electricity, supplying an indifferent gas as a pressure medium, releasing the pressure to produce a partial vacuum and finally increasing the same, substantially as and for the purposes described.

7. In a process of casting molten metals under pressure, which consists in heating a metal bath internally by means of electricity, suddenly releasing the pressure to produce a partial vacuum in the melting chamber and then increasing the same, substantially as and for the purposes described.

8. In a process of casting molten metals under pressure, which consists in heating a metal bath internally by means of electricity, suddenly releasing the pressure to produce a partial vacuum in the melting chamber and increasing the vacuum by connecting the chamber with a vacuum pipe, substantially as and for the purposes described.

9. In a process of casting molten metals under pressure, which consists of internally heating a metal bath held in a gas-tight condition under pressure, releasing the pressure and establishing a vacuum in the chamber in which the metal bath is held and then increasing the vacuum thus created, substantially as and for the purposes described.

In testimony, that I claim the foregoing as my invention, I have signed my name in presence of two subscribing witnesses.

FRANZ DE BUIGNÉ.

Witnesses:

WOLDEMAR HAUPT,  
HENRY HASPER.